

## [54] INHIBITION OF CORROSION

[75] Inventors: **Winston Costain; Bernard William Hugh Terry**, both of Blackley, England

[73] Assignee: **Imperial Chemicals Industries Limited**, London, England

[22] Filed: Jan. 24, 1974

[21] Appl. No.: 436,351

## Related U.S. Application Data

[63] Continuation of Ser. No. 180,231, Sept. 13, 1971, abandoned.

## [30] Foreign Application Priority Data

Sept. 24, 1970 United Kingdom..... 45814/70  
Mar. 25, 1971 United Kingdom..... 7807/71

[52] U.S. Cl..... 21/2.5 R; 21/2.7 R; 252/148; 252/390; 252/392; 252/394

[51] Int. Cl..... C23f 11/04; C23f 11/14

[58] Field of Search..... 21/2.5 R, 2.7 R; 252/148, 252/390, 392, 394

## [56] References Cited

## UNITED STATES PATENTS

|           |         |                    |             |
|-----------|---------|--------------------|-------------|
| 2,043,260 | 6/1936  | Missbach.....      | 21/2.5 R UX |
| 2,239,752 | 4/1941  | Lewis.....         | 252/392 X   |
| 2,387,323 | 10/1945 | Gaynor et al. .... | 252/392 X   |
| 2,700,652 | 1/1955  | Menaul.....        | 21/2.5 R X  |
| 2,863,837 | 12/1958 | Kowald et al. .... | 252/394     |

|           |        |                       |            |
|-----------|--------|-----------------------|------------|
| 3,031,411 | 4/1962 | Petering et al.....   | 252/392 X  |
| 3,081,304 | 3/1963 | Rogier.....           | 21/2.7 R X |
| 3,096,147 | 7/1963 | Fulmer.....           | 21/2.7 R   |
| 3,096,341 | 7/1963 | Sheppard et al.....   | 252/390 X  |
| 3,098,700 | 7/1963 | Bernard.....          | 21/2.7 R   |
| 3,255,121 | 6/1966 | Riggs.....            | 21/2.7 R X |
| 3,553,101 | 1/1971 | Foroulis.....         | 21/2.7 R X |
| 3,658,720 | 4/1972 | McDougall et al. .... | 21/2.7 R X |
| 3,669,612 | 6/1972 | Annand et al. ....    | 21/2.5 R   |

## FOREIGN PATENTS OR APPLICATIONS

|          |         |            |         |
|----------|---------|------------|---------|
| 38/26754 | 12/1963 | Japan..... | 252/394 |
|----------|---------|------------|---------|

## OTHER PUBLICATIONS

Betz; Handbook of Industrial Water Conditioning; 6th Edition, 1962, Phila., Pa., pp. 276-278.

Chemical Abstracts; Vol. 46, No. 11, 4983h, June, 1952 "Action of Inhibitors in Pickling"; Indelli et al.

Primary Examiner—Barry S. Richman

Attorney, Agent, or Firm—Cushman, Darby & Cushman

## [57] ABSTRACT

A method of inhibiting the corrosion of steel by acidic compounds, which comprises adding to the acidic compound an organic nitrogen compound containing at least one unsaturated carbon-nitrogen bond (other than a cyclic vicinal dinitrile) or by pre-treatment of the steel with the organic nitrogen compound or by a combination of both methods.

5 Claims, No Drawings

## INHIBITION OF CORROSION

This is a continuation, of application Ser. No. 180,231 filed Sept. 13, 1971, now abandoned.

This invention relates to the inhibition of the corrosion of steel by acids, and more particularly to the use of certain organic nitrogen compounds as corrosion inhibitors.

Steel is widely used as material of construction, particularly for chemical plant, and is consequently subjected to attack by a wide variety of corrosive substances, including organic and inorganic acids. Such corrosion presents serious problems, for not only is the structure itself attacked by contact with corrosive substances, thereby making necessary more frequent maintenance and replacement of expensive equipment than would otherwise be the case, but the products made in, for example the chemical plant are contaminated by material resulting from such corrosive attack.

We have found that the corrosion of steel by organic and inorganic acids is inhibited by the addition to the acid of an effective amount of an organic nitrogen compound containing at least one unsaturated carbon-nitrogen bond, or by pre-treatment of the steel with the said organic nitrogen compound, or by a combination of both methods, provided that the organic nitrogen compound is other than a cyclic vicinal dinitrile.

As examples of organic compounds containing at least one unsaturated carbon-nitrogen bond which may be used as corrosion inhibitors according to the present invention there may be mentioned those classes of compounds containing one or more nitrile, isonitrile, oxime, hydrazone, amidine, amidoxime, semicarbazone, hydrazone or imine group, the latter class including groups which form part of a heterocyclic ring system as in, for example, oxazoles, oxadiazoles, furazans, furoxans, iminazoles, pyrazoles, pyrazolones, pyrazolines and triazoles.

Suitable compounds include acrylonitrile and substituted acrylonitriles, for example, crotononitrile, cinnamonnitrile, p-methoxycinnamonnitrile and 1-cyano-4-phenylbuta-1,3-diene; benzonitriles and naphthonitriles carrying non-ionised electron-donating groups, for example, hydroxy, alkoxy, alkyl, halogen, trihalogenomethyl, thiol and thioether groups, specific examples of which include p-chloro-benzonitrile, p-methoxybenzonitrile, p-dodecylbenzonitrile, p-trichloromethylbenzonitrile, m-tolunitrile and 1-cyano-4-methoxy-naphthalene; other substituted benzonitriles, including p-nitro-benzonitrile, p-dimethylaminobenzonitrile, and p-aminobenzonitrile; N,N,N',N'-tetrakis-(cyanomethyl)hexamethylenediamine, N,N'-bis(α-cyano-benzyl)ethylenediamine, diphenylmethane nitriles, for example, 3,3'-dicyanodiphenylmethane, diphenylnitriles, for example, 4,4'-dicyanodiphenyl, naphthylnitriles, for example, 1-cyanophthalene; o- and p-cyanobenzaldehyde, 2-pentenonitrile, cyanoacetic acid, cyanovaleric acid, cyanocaproic acid, 2-, 3- and 4-cyanopyridines, alkyl nitriles, for example, octadecanonitrile, succinonitrile, adiponitrile, azelaonitrile, sebaconitrile, decane-1,10-dicarbonitrile, dodecane dinitrile, 1,4-dicyanobutene-2, 1,4-bis(-cyanoethoxy)-butyne-2, fumaronitrile, maleonitrile, phenylmaleonitrile, acetonitrile and substituted acetonitriles, for example, benzyl cyanide, diphenylacetonitrile and triphenylacetonitrile; 2-cyanocyclopentylideneimine, dimethyl glyoxime, cyclohexanoneoxime, 1,2- and 1,4-cyclohexane diketox-

ime, acetoxime, benzalacetoxime; dibenzalacetoxime, benzamideoxime, o- and p-benzoquinone monoximes and dioximes, acetophenoneoxime, benzophenoneoxime, benzaldoxime, cinnamaldoxime, guanidine salts, for example, guanidine carbonate, pyridine, 2,2'-bipyridyl, 4,4-bipyridyl, quinoline, isoquinoline, 1-cyanoisoquinoline, benzofurazan, cyclohexylfurazan, benzofuroxan, cyclohexylfuroxan, pyridine-N-oxide and substituted pyridine-N-oxides, benzoxazone, benzimidazole and metal-free phthalocyanines.

Polymers and iron-complexing agents such as bipyridyl, ethylene diamine diacetic acid, phenanthrolines, quinolines and isoquinolines containing unsaturated carbon-nitrogen groupings as defined above are also satisfactory. Mixtures of inhibitors according to the present invention may also be used for wider effects, as synergists or as compositions having a wide vapour pressure range. The compounds are also effective when used together with copper cyanide.

A preferred class of compounds, particularly effective in protecting mild steels as well as stainless steels against acid attack, consists of conjugated unsaturated nitriles. As examples of such compounds there may be mentioned 1-cyano-4-pyrimidin-2'-ylbuta-1,3-diene, 1-cyanobut-1-ene-3-yne, 1-cyanohexa-1,5-diene-3-yne and 6-cyanohexa-1,3,5-triene-1-yl dimethyl phenyl ammonium salts, for example, the chloride, bromide, iodide, methosulphate or ethosulphate, but preferred compounds in this class are cinnamonitrile, p-methoxy-cinnamonitrile, crotononitrile and 1-cyano-4-phenylbuta-1,3-diene.

A second preferred class of compounds, also particularly effective in inhibiting acid attack on mild steel, consists of conjugated unsaturated oximes, of which preferred compounds are cinnamaldoxime, benzalacetoxime and dibenzalacetoxime.

As examples of organic acids against the corrosive attack of which the above compounds are effective there may be mentioned monocarboxylic acids such as formic acid, acetic acid, propionic acid, n-butyric acid, isobutyric acid, stearic acid, monochloro-, dichloro- and trichloroacetic acids and the corresponding bromoacetic acids, lactic acid, dicarboxylic acids such as oxalic acid, succinic acid, glutaric acid, adipic acid, pimelic acid, terephthalic acid, suberic acid, azelaic acid, sebatic acid, undecanedioic and dodecanedioic acid, tartaric acid and tricarboxylic acids such as citric acid and trimesic acid.

The method of the present invention is also effective against attack by organic sulphonic acids.

As examples of inorganic acids, the corrosive effects on steel of which are minimised according to the invention, there may be mentioned aqueous sulphurous acid, sulphuric acid, aqueous solutions of hydrogen halides, e.g., hydrochloric acid, sulphamic acid and nitric acid.

The method is also effective against the corrosion of steels by derivatives of acids which may undergo chemical reaction with consequent liberation of the free acids, for example, anhydrides, esters and amides in the case of carboxylic acids and is applicable both to the anhydrous acids and aqueous solutions thereof.

The corrosion-inhibiting compounds used according to the present invention are effective at temperatures from ambient temperature or below up to 240°C or even higher.

By 'an effective amount' we mean an amount of the organic nitrogen compound which is effective in inhibiting corrosion under the prevailing conditions.

In the case where the inhibitor is added to the organic or inorganic acid an amount of inhibitor from a trace up to 10 percent by weight, more usually up to 5 percent by weight, based on the weight of acid, is generally effective.

Pre-treatment of steel with the inhibitor compound may be carried out using the compound neat, as vapour or as a solution in a suitable solvent, for example water, alcohols, acids, bases such as pyridine and quinoline, and nitriles and at temperatures up to 300°C.

The inhibitor compounds may also be incorporated in paints, primers, and wax or polish compositions intended for application to steel and in impregnated interlining and packing materials such as paper intended for wrapping and protecting steel. The inhibitor compounds may also be used as corrosion inhibitors in acid pickling baths which are employed in removing oxide scale from ferrous metals, and these uses form further features of the invention.

A wide variety of steels may be protected against corrosion using the methods described above, for example, stainless steels of American Iron and Steel Institute

Types 304, 316 and 321 (the compositions of which are defined in, for example, British Standard No. 1449, part 4, page 20) and mild steels. The corrosion-inhibiting organic nitrogen compounds hereinbefore described are also effective in protective steels from attack by high performance (jet) lubricants. The invention is illustrated but not limited by the following Examples.

10

4

#### EXAMPLE 1-27

A weighed rectangular prism of steel, 25-35 g. in weight, stamped and drilled with an 0.375 inch hole, was placed in a 8 × 1 inch glass tube (fitted with air and water reflux condensers) together with adipic acid (30 g), inhibitor (1g. of a solid or 1 ml. of a liquid) and distilled water (1 ml.). The mixture was heated in a Wood's Metal bath at 240° ± 10°C for 50 hours and the sample was removed, washed, dried, weighed and its appearance noted. Some samples were given a preliminary treatment by heating for 1 hour with a 2 percent w/v solution of inhibitor in an appropriate solvent at the boil and then allowed to cool during 24 hours before testing.

20 Results are given in the following table.

| Exam-<br>ple | Type of Steel             | INHIBITOR                          | Weight<br>loss<br>ppm | REMARKS                                                                                                                                                    |
|--------------|---------------------------|------------------------------------|-----------------------|------------------------------------------------------------------------------------------------------------------------------------------------------------|
| 1.           | Stainless Type 321<br>do. | None (Control)<br>Adiponitrile     | 10,165<br>38          | Severe general corrosion<br>Undrilled sample. Bright metal<br>surface unchanged on exposure.<br>Slight pitting on edges                                    |
| 2.           | do.                       | succinonitrile                     | 160                   | surface slightly dulled on exposure                                                                                                                        |
| 3.           | do.                       | 2-cyano cyclopentyl-<br>ideneimine | 32                    | bright surface unchanged                                                                                                                                   |
| 4.           | do.                       | cyclohexane 1,2-dione<br>dioxime   | 64                    | Bright surface unchanged                                                                                                                                   |
| 5.           | do.                       | cyclohexanone oxime                | 11                    | Bright surface unchanged                                                                                                                                   |
| 6.           | do.                       | o benzoquinone dioxime             | 15                    | do.                                                                                                                                                        |
| 7.           | do.                       | p benzoquinone dioxime             | 24                    | do.                                                                                                                                                        |
| 8.           | do.                       | benzaldoxime                       | 234                   | Surface dulled and slight corrosion                                                                                                                        |
| 9.           | do.                       | Benzofuroxan                       | 15                    | Bright surface unchanged                                                                                                                                   |
| 10.          | do.                       | 22' Bipyridyl                      | 0                     | Sample pretreated prior to testing                                                                                                                         |
| 11.          | do.                       | Dimethyl glyoxime                  | 1,050                 | Corrosion round hole and stamping-<br>some pitting on sides                                                                                                |
| 12.          | do.                       | Guanidine carbonate                | 43                    | Bright surface retained. Slight<br>evidence of pitting.                                                                                                    |
| 13.          | do.                       | Fumaronitrile                      | 440                   | Some dulling on edges. Slight pitting                                                                                                                      |
| 14.          | do.                       | Acetonitrile                       | 1,975                 | General corrosion - less than control                                                                                                                      |
| 15.          | do.                       | Cyano acetic acid                  | 2,267                 | do.                                                                                                                                                        |
| 16.          | do.                       | phthalonitrile                     | 4,135                 | Severe general corrosion                                                                                                                                   |
| 17.          | do.                       | metal free phthalo-<br>cyanine     | 49                    | Sample pretreated in inhibitor in<br>quinoline solvent in addition to that<br>added in normal test. Slight tarnish-<br>no pitting                          |
| 18.          | do.                       | Cuprous cyanide                    | 2,604                 | General corrosion                                                                                                                                          |
| 19.          | do.                       | Cuprous cyanide +<br>adiponitrile  | 26.5                  | Sample pretreated with inhibitors<br>Inhibitors present during test-<br>slight bloom on sample                                                             |
| 20.          | do.                       | Cyclohexane-1,2-dione<br>dioxime   | 646                   | Sample pretreated with inhibitor in<br>ethyl alcohol. No inhibitor in test.<br>Surfaide of sample after test generally<br>bright - some areas of corrosion |
| 21.          | Mild steel<br>do.         | —                                  | 57,500                | Severe general corrosion                                                                                                                                   |
| 22.          |                           | Cyclohexane 1,2-dione<br>dioxime   | 25,400                | General corrosion. Sample surface<br>smoother than control. Corrosion less<br>severe than control                                                          |
| 23.          | Stainless Type 321<br>do. | Pyridine N-oxide                   | 10                    | Bright surface unchanged                                                                                                                                   |
| 24.          |                           | 2-cyano pyridine                   | 26                    | do.                                                                                                                                                        |
| 25.          |                           | Acetoxime                          | 19                    | do.                                                                                                                                                        |
| 26.          |                           | Acetophenoneoxime                  | 0                     | do.                                                                                                                                                        |
| 27.          |                           | Benzamidoxime                      | 7.5                   | do.                                                                                                                                                        |

## EXAMPLES 28-44

A rectangular steel strip (Stainless Type 321), 8-9g. in weight, approximately,  $1.5 \times 0.75 \times 0.0625$  inch, drilled with a 0.375 inch diameter hole, is placed in a  $8 \times 1$  inch glass tube fitted with air-cooled and water-cooled reflux condensers, together with the acid (50 ml) under test and is then heated at the temperatures and for the times indicated in the following table. The inhibitor was added to the acid solution at a concentration of 2 percent w/v. The metal samples were weighed before and after exposure to the acid.

## EXAMPLES 48-55

A rectangular mild steel strip, - 3.5 g. in weight, approximately  $2 \times \frac{5}{8} \times \frac{1}{32}$  inch is placed in an  $8 \times 1$  inch test-tube fitted with air and water-cooled condensers in series, together with 16 w/w hydrochloric acid

(50 ml) to which the inhibitor is added and is then heated at  $80^\circ \pm 1^\circ\text{C}$  for the times indicated in the following table. The metal samples were weighed before and after exposure to the acid.

5

## EXAMPLES 56-82

A bright metal steel rectangular ticket,  $2 \times \frac{5}{8} \times \frac{1}{32}$  inch, was immersed in 25 ml 16 w/w percent hydrochloric acid containing approximately 2 percent w/v of inhibitor in a  $6 \times 1$  inch boiling tube and boiled for 10-20 seconds. Gas evolution was initiated in the boiling acid by contact of the mild steel ticket with an aluminum rod and the tube and contents were then allowed to cool during 15 minutes. The hydrogen evolution rate and the final appearance of the metal sample were noted.

| Example | Acid                       | INHIBITOR                  | Time (hours) | Temp. (°C) | Weight Loss |
|---------|----------------------------|----------------------------|--------------|------------|-------------|
| 28      | 98 % acetic acid           | None (Control)             | 100          | 120        | 2600 p.p.m. |
| 29      | do.                        | Nioxime                    | 100          | 120        | 33 do.      |
| 30      | do.                        | Benzimidazole              | 100          | 120        | 65 do.      |
| 31      | do.                        | Cyclohexanone oxime        | 100          | 120        | 0 do.       |
| 32      | do.                        | Benzofuroxan               | 100          | 120        | 23 do.      |
| 33      | do.                        | None (Control)             | 100          | 120        | 3400 do.    |
| 34      | 90 % Formic acid           | None (Control)             | 100          | 100        | 5460 do.    |
| 35      | do.                        | Cyclohexanone oxime        | 100          | 100        | 63 do.      |
| 36      | do.                        | None (Control)             | 100          | 100        | 6500 do.    |
| 37      | 20 % Sulphuric acid        | None (Control)             | 72           | 80         | 10.7%       |
| 38      | do.                        | Cyclohexanone oxime        | 72           | 80         | 2.1%        |
| 39      | do.                        | 2-cyanopyridine            | 72           | 80         | 1.2%        |
| 40      | do.                        | Acetoxime                  | 72           | 80         | 1.3%        |
| 41      | do.                        | None (Control)             | 72           | 80         | 8.3%        |
| 42      | 14 % w/v Hydrochloric acid | None (Control)             | 24           | 86         | 29.8%       |
| 43      | do.                        | 2-cyanopyridine            | 24           | 80         | 5.1%        |
| 44      | do.                        | None (Control)             | 24           | 80         | 29.6%       |
| 45      | do.                        | 1-cyano-4-phenyl butadiene | 24           | 80         | 0.013%      |
| 46      | do.                        | cinnamaldoxime             | 24           | 80         | 0.04%       |
| 47      | do.                        | cinnamonnitrile            | 24           | 80         | 0.013%      |

| Example | INHIBITOR                     | EXPOSURE AT 80°C |                       |                       |                        |
|---------|-------------------------------|------------------|-----------------------|-----------------------|------------------------|
|         |                               | Compound         | Conc. in acid (% w/v) | 4 hours weight loss % | 24 hours weight loss % |
| 48      | Benzonitrile                  |                  | 0.2                   | 24.5                  | Dissolved              |
| 49      | Dodecane dinitrile            |                  | 0.2                   | 3.2                   | 9.2                    |
| 50      | Fumaronitrile                 |                  | 0.2                   | 6.0                   | 43.0                   |
| 51      | p-methoxybenzonitrile         |                  | 0.2                   | 0.67                  | 1.9                    |
| 52      | 1-cyano-4-methoxy naphthalene |                  | 0.2                   | 0.34                  | 0.72                   |
| 53      | p-dodecylbenzonitrile         |                  | 0.2                   | 2.6                   | 5.9                    |
| 54      | cinnamonnitrile               |                  | 0.1                   | 0.15                  | 0.47                   |
| 55      | Control                       |                  | NIL                   | Dissolved             | Dissolved              |

| Example | INHIBITOR                                            | Hydrogen Evolution Rate    | Appearance of metal after exposure. |
|---------|------------------------------------------------------|----------------------------|-------------------------------------|
| 56      | benzyl cyanide                                       | practically nil            | no apparent change                  |
| 57      | N,N,N',N'-tetrakis-(cyanomethyl)hexamethylenediamine | do.                        | do.                                 |
| 58      | octadecyl cyanide                                    | do.                        | do.                                 |
| 59      | 1-cyanoisoquinoline                                  | do.                        | do.                                 |
| 60      | 1-cyanonaphthalene                                   | do.                        | do.                                 |
| 61      | 4,4'-dicyanodiphenyl                                 | do.                        | do.                                 |
| 62      | 3,3'-dicyanodiphenylmethane                          | do.                        | do.                                 |
| 63      | p-chlorobenzonitrile                                 | do.                        | do.                                 |
| 64      | acrylonitrile                                        | do.                        | do.                                 |
| 65      | 2-pentenenitrile                                     | do.                        | do.                                 |
| 66      | phenylmaleonitrile                                   | do.                        | do.                                 |
| 67      | p-trichloromethyl benzonitrile                       | do.                        | do.                                 |
| 68      | m-toluonitrile                                       | do.                        | do.                                 |
| 69      | p-nitrobenzonitrile                                  | fast & continuous          | dull & corroded                     |
| 70      | p-dimethylaminobenzonitrile                          | do.                        | do.                                 |
| 71      | p-aminobenzonitrile                                  | Fairly slow but continuous | dulled                              |
| 72      | p-cyanobenzaldehyde                                  | slow but continuous        | dulled                              |
| 73      | o-cyanobenzaldehyde                                  | fairly slow but continuous | dulled                              |
| 74      | N,N'-bis( $\alpha$ -cyanobenzyl)ethylenediamine      | very slow                  | bright                              |
| 75      | cinnamonnitrile                                      | practically nil            | no apparent change                  |
| 76      | p-methoxy cinnamonnitrile                            | do.                        | do.                                 |
| 77      | 1-phenyl-4-cyano butadiene                           | do.                        | do.                                 |
| 78      | crotononitrile                                       | do.                        | do.                                 |
| 79      | cinnamaldoxime                                       | do.                        | do.                                 |
| 80      | benzalacetoxime                                      | do.                        | do.                                 |
| 81      | benzalacetoxime                                      | do.                        | do.                                 |
| 82      | none (Control)                                       | very fast and continuous   | dull and severely corroded          |

We claim:

1. A method of inhibiting the corrosion of steel by acidic compounds which comprises adding to the acidic compound an effective amount of a compound selected from the group consisting of nitriles, aldoximes and ketoximes, wherein the nitrile is further selected from the group consisting of nitriles in which the nitrile group is attached to an unsaturated aliphatic carbon chain to form a conjugated system including the nitrile group and at least two double bonds in the chain, 10 and nitriles in which the nitrile group is attached to an unsaturated aliphatic carbon chain which is itself attached to a benzene nucleus to form a conjugated system including the nitrile group, the benzene nucleus and at least one double bond in the unsaturated aliphatic carbon chain; and wherein the aldoximes and ketoximes are further selected from the group consisting of orthobenzene quinone dioxime, parabenzoylquinone dioxime, aldoximes and ketoximes in which the oxime group is directly attached to a benzene nucleus 15 and aldoximes and ketoximes in which the oxime group

5

10

15

20

15

20

is attached to a benzene nucleus through an unsaturated aliphatic carbon chain to form a conjugated system including the benzene nucleus, the oxime group and at least one double bond in the unsaturated aliphatic carbon chain.

2. A method as claimed in claim 1 wherein the acidic compound is a carboxylic acid.

3. A method as claimed in claim 1 wherein the acidic compound is an organic sulphonate acid or an inorganic acid.

4. A method as claimed in claim 1 wherein the corrosion inhibiting compound is a conjugated unsaturated nitrile selected from the group consisting of cinnamonnitrile, p-methoxy-cinnamonnitrile, phenylmaleonitrile and 1-cyano-4-phenylbuta-1,3-diene.

5. A method as claimed in claim 1 wherein the corrosion inhibiting compound is a conjugated unsaturated oxime selected from the group consisting of cinnamaldoxime, benzalacetoxime, acetophenoneoxime and dibenzalacetoxime.

\* \* \* \* \*

25

30

35

40

45

50

55

60

65